

1

3,118,763

**COBALT BASE ALLOYS**

Rudolf H. Thielemann, Palo Alto, Calif., assignor to Sierra Metals Corporation, Chicago, Ill., a corporation of Delaware

No Drawing. Filed July 28, 1958, Ser. No. 751,159

9 Claims. (Cl. 75—171)

This invention relates to a cobalt base metal alloy which includes alloying metal additives which make the resulting alloy corrosion resistant and of great mechanical work strength at temperatures between about 1500° F. and about 2200° F.

Important features of the alloy of this invention are that it may be cast, is highly resistant to oxidation and other forms of corrosion, and possesses great mechanical strength at temperatures up to between about 1500° F. and about 2200° F. As a result, this alloy may be used as blades, vanes, and other parts of high temperature gas turbine engines. Other important uses of the alloy of this invention are as exhaust valves and manifolds in internal combustion engines, heat exchanges, as linings for retorts and container vessels used in the chemical and metallurgical industries, and as an oxidation resistant coating material for metals and metal alloys such as columbium, tantalum, nickel base alloys, cobalt base alloys, etc., which possess high strength characteristics at elevated temperatures but whose resistance to oxidation at elevated temperatures, i.e., above about 1500° F., is inadequate. The alloy of this invention can also be utilized as high temperature, high strength, corrosion resistant tubing and sheet material, as a material for forming cutting blades useful for cutting molten glass and other hot corrosive materials, as a material for forming supporting members or holders for use in metallurgical testing apparatus, etc.

The prior art nickel and/or cobalt base metal alloys which have been used as blades, vanes, and other parts of high temperature gas turbine engines, have a maximum operating temperature of about 1500° F. For example, a common nickel-cobalt base metal alloy which incorporates molybdenum as a constituent is for all practical purposes non-utilizable as a structural member in a gas turbine engine if the metal temperature is above 1500° F. One reason for this temperature limit is that the oxidation resistance of such an alloy fails above 1500° F.

An alloy of this invention when used as a blade or vane in a high temperature gas turbine engine can be operated at markedly higher temperatures than was possible heretofore. The performance of gas turbine engines incorporating such blades or vanes is considerably improved, since at higher temperatures the total thrust of a gas turbine engine increases and the amount of fuel consumed per pound of thrust decreases.

The metal alloy of this invention is comprised, by weight, of the following constituents: from about 15 to about 28 percent of chromium; from about 5 to about 15 percent of tungsten; from about 0.5 to about 20 percent of tantalum; from about 0.01 to about 3 percent of titanium; from about 0.1 to about 1.3 percent of carbon; and the balance being essentially cobalt.

I have found that the high temperature corrosion resistant properties of the alloy of this invention are not

2

affected if the alloy includes an amount of columbium which is not more than one-half of the amount of tantalum in the alloy and, in any event, is no greater than 3 percent, by weight, of the alloy, and preferably not more than 2.0 percent, by weight, of the alloy.

It is important to note that in the past the metals tantalum and columbium have been considered to be equivalent for various purposes. This is not true in the case of the alloy of this invention. For example, if in the alloy of this invention, columbium is substituted for tantalum in the range of proportions specified, the resulting alloy does not possess the high temperature corrosion resistance characteristic of the alloy of this invention.

While molybdenum is not a primary constituent of the alloy of this invention, I have found that the properties of the alloy of this invention are not deleteriously affected if the alloy includes an amount of molybdenum which is not more than one-half the amount of tungsten in the alloy and, in any event, is no greater than 3.5 percent, by weight, of the alloy.

I have also found that zirconium may be tolerated in the alloy of this invention in an amount such that if the amount of titanium in the alloy is more than about 0.5 percent, the combined amount of titanium and zirconium is equal to or less than about 3 percent, and if the amount of titanium is equal to or less than about 0.5 percent, the amount of titanium is more than about 70 percent of the amount of zirconium in the alloy.

It has been further found that the inclusion of any one or more of the following ingredients: up to about 0.2 percent of boron, up to about 1.5 percent of silicon, and up to about 5 percent of nickel and/or iron may in certain formulations improve various metallurgical characteristics of the alloy. Additional amounts of these ingredients may in some cases be tolerated in the alloy without deleterious effects.

It is to be noted that if the boron content in the alloy of this invention exceeds about 0.2 percent, then the alloy of this invention becomes unsatisfactory, particularly in those applications where thermal shock requirements are important.

To achieve the optimum desired properties, it is preferred that the following impurities which may be in the alloy be held to the following limits by weight. The manganese content in the final alloy should not be greater than about 2 percent. The interstitial elements such as nitrogen, hydrogen, tin, lead, and the like should be kept as low as possible. In addition, not more than about 0.5 percent total of deoxidizers such as calcium, magnesium, and the like should be present in the final alloy.

A preferred range of proportions of constituents of the alloy of this invention which has especially high oxidation resistance and strength characteristics, at temperatures of 2000° F., and above, and which is particularly suitable for use as a vane material in a gas turbine, high temperature engine is as follows: from about 16 to about 25 percent of chromium; from about 7.5 to about 12.5 percent of tungsten; from about 7 to about 11 percent of tantalum; from about .08 to about 0.5 percent of titanium; from about 0.6 to about 1.0 percent of carbon; and the balance being essentially cobalt.

Following are examples of the preparation and test results of the cobalt base metal alloy of this invention.

*Example 1*

A 5 pound alloy melt of a cobalt base metal alloy composition containing about 20 percent of chromium, about 11 percent of tungsten, about 1.5 percent of tantalum, about 1.5 percent of titanium, about 0.1 percent of carbon, and the balance essentially cobalt, all percentages by weight, was prepared by melting the chromium and cobalt in a magnesia crucible under high vacuum conditions, following which the tungsten, tantalum, titanium, and carbon in the form of graphite were added.

A cluster of 6 test bars were formed from the 5 pound melted alloy heat and cast by the usual investment casting technique under high vacuum conditions. These bars were each 3 inches long and  $\frac{1}{4}$  inch in diameter.

The test bars of this example had an elongation of 10 percent at room temperature under a tensile stress of 95,000 p.s.i.

The test bars of this example had a rupture life in excess of 100 hours under a load of 12,000 p.s.i. at a temperature of about 1700° F. in air and a rupture life in excess of 100 hours under a load of 10,000 p.s.i. at a temperature of about 1800° F. in air.

*Example 2*

A 5 pound alloy melt and test bars of the same dimensions as set forth in Example 1 of a cobalt base metal alloy composition containing about 28 percent of chromium, about 5 percent of tungsten, about 1.5 percent of tantalum, about 1.5 percent of titanium, about 0.4 percent of carbon, and the balance essentially cobalt, all percentages by weight, were prepared in the same manner as set forth in Example 1.

The test bars of this example had an elongation of 3 percent at room temperature under a tensile stress of 100,000 p.s.i.

The test bars of this example had a rupture life in excess of 100 hours under a load of 15,000 p.s.i. at a temperature of about 1700° F. in air and a rupture life in excess of 100 hours under a load of 8,000 p.s.i. at a temperature of about 1800° F. in air.

*Example 3*

A 5 pound alloy melt and test bars of the same dimensions as set forth in Example 1 of a cobalt base metal alloy composition containing about 20 percent of chromium, about 11 percent of tungsten, about 0.5 percent of tantalum, about 3 percent of titanium, about 0.7 percent of carbon, and the balance essentially cobalt, all percentages by weight, were prepared in the same manner as set forth in Example 1.

The test bars of this example had an elongation of 7 percent at room temperature under a tensile stress of 115,000 p.s.i.

The test bars of this example had a rupture life in excess of 100 hours under a load of 15,000 p.s.i. at a temperature of about 1700° F. in air and a rupture life in excess of 100 hours under a load of 10,000 p.s.i. at a temperature of about 1800° F. in air.

*Example 4*

A 5 pound alloy melt and test bars of the same dimensions as set forth in Example 1 of a cobalt base metal alloy composition containing about 20 percent of chromium, about 10 percent of tungsten, about 10 percent of tantalum, about 0.3 percent of titanium, about 1.0 percent of carbon, and the balance essentially cobalt, all percentages by weight, were prepared in the same manner as set forth in Example 1.

The test bars of this example had an elongation of 3 percent at room temperature under a tensile stress of 118,000 p.s.i.

The test bars of this example had a rupture life in excess of 100 hours under a load of 25,000 p.s.i. at a temperature of about 1600° F. in air, a rupture life in

excess of 100 hours under a load of 18,000 p.s.i. at a temperature of about 1700° F. in air, and a rupture life in excess of 100 hours under a load of 12,000 p.s.i. at a temperature of about 1800° F. in air.

*Example 5*

A 5 pound alloy melt and test bars of the same dimensions as set forth in Example 1 of a cobalt base metal alloy composition containing about 15 percent of chromium, about 15 percent of tungsten, about 13 percent of tantalum, about 0.01 percent of titanium, about 0.65 percent of carbon, and the balance essentially cobalt, all percentages by weight, were prepared in the same manner as set forth in Example 1.

The test bars of this example had an elongation of 5 percent at room temperature under a tensile stress of 124,000 p.s.i.

The test bars of this example had a rupture life in excess of 100 hours under a load of 25,000 p.s.i. at a temperature of about 1600° F. in air, a rupture life in excess of 100 hours under a load of 18,000 p.s.i. at a temperature of about 1700° F. in air, and a rupture life in excess of 100 hours under a load of 10,000 p.s.i. at a temperature of about 1800° F. in air.

*Example 6*

A 5 pound alloy melt and test bars of the same dimensions as set forth in Example 1 of a cobalt base metal alloy composition containing about 20 percent of chromium, about 10 percent of tungsten, about 20 percent of tantalum, about 2 percent of titanium, about 1 percent of zirconium, about 0.85 percent of carbon, and the balance essentially cobalt, all percentages by weight, were prepared in the same manner as set forth in Example 1.

The test bars of this example had an elongation of 6 percent at room temperature under a tensile stress of 118,000 p.s.i.

The test bars of this example had a rupture life in excess of 100 hours under a load of 20,000 p.s.i. at a temperature of about 1600° F. in air, a rupture life in excess of 100 hours under a load of 15,000 p.s.i. at a temperature of about 1700° F. in air, and a rupture life in excess of 100 hours under a load of 8,000 p.s.i. at a temperature of about 1800° F. in air.

*Example 7*

A 5 pound alloy melt and test bars of the same dimensions as set forth in Example 1 of a cobalt base metal alloy composition containing about 28 percent of chromium, about 5 percent of tungsten, about 8 percent of tantalum, about 2.0 percent of titanium, about 0.5 percent of zirconium, about 0.7 percent of carbon, and the balance essentially cobalt, all percentages by weight, were prepared in the same manner as set forth in Example 1.

The test bars of this example had an elongation of 1 percent at room temperature under a tensile stress of 120,000 p.s.i.

The test bars of this example had a rupture life in excess of 100 hours under a load of 20,000 p.s.i. at a temperature of about 1600° F. in air, a rupture life in excess of 100 hours under a load of 10,000 p.s.i. at a temperature of about 1700° F. in air, and a rupture life in excess of 100 hours under a load of 5,000 p.s.i. at a temperature of about 1800° F. in air.

*Example 8*

A 5 pound alloy melt and test bars of the same dimensions as set forth in Example 1 of a cobalt base metal alloy composition containing about 21.3 percent of chromium, about 9.7 percent of tungsten, about 2.7 percent of tantalum, about 0.2 percent of zirconium, about 0.2 percent of titanium, about 0.45 percent of carbon, about 0.4 percent of silicon, about 0.28 percent of manganese, about 0.5 percent of nickel, about 0.5 percent of iron, and the balance essentially cobalt, all percentages by

weight, were prepared in the same manner as set forth in Example 1.

The test bars of this example had an elongation of about 2 percent at room temperature under a tensile stress of 113,000 p.s.i.

The test bars of this example had a rupture life in excess of 250 hours under a load of 22,000 p.s.i. at a temperature of about 1600° F. in air, a rupture life of about 329 hours under a load of 15,500 p.s.i. at a temperature of about 1700° F., and a rupture life in excess of 63 hours under a load of 8,000 p.s.i. at a temperature of about 1800° F. in air.

#### Example 9

A 5 pound alloy melt and test bars of the same dimensions as set forth in Example 1 of a cobalt base metal alloy composition containing about 21.5 percent of chromium, about 9.6 percent of tungsten, about 1.2 percent of tantalum, about 0.3 percent of titanium, about 0.45 percent of carbon, about 1.5 percent of silicon, about 0.28 percent of manganese, about 1.5 percent of nickel, about 1.5 percent of iron, and the balance essentially cobalt, all percentages by weight, were prepared in the same manner as set forth in Example 1.

The test bars of this example had an elongation of about 3.3 percent at room temperature under a tensile stress of 118,000 p.s.i.

The test bars of this example had a rupture life in excess of 233 hours under a load of 13,000 p.s.i. at a temperature of about 1700° F. in air, and a rupture life in excess of 154 hours under a load of 10,000 p.s.i. at a temperature of about 1800° F. in air.

#### Example 10

A 5 pound alloy melt and test bars of the same dimensions as set forth in Example 1 of a cobalt base metal alloy composition containing about 21.5 percent of chromium, about 9.7 percent of tungsten, about 10.6 percent of tantalum, about 0.4 percent of zirconium, about 0.3 percent of titanium, about 0.75 percent of carbon, and the balance essentially cobalt, all percentages by weight, were prepared in the same manner as set forth in Example 1.

The test bars of this example had an elongation of 1.1 percent at room temperature under a tensile stress of 110,000 p.s.i.

The test bars of this example had a rupture life in excess of 59 hours under a load of 17,000 p.s.i. at a temperature of about 1800° F. in air.

#### Example 11

A 5 pound alloy melt and test bars of the same dimensions as set forth in Example 1 of a cobalt base metal alloy composition containing about 21 percent of chromium, about 9 percent of tungsten, about 9 percent of tantalum, about 0.2 percent of titanium, about 0.85 percent of carbon, about 1.0 percent of molybdenum, and the balance essentially cobalt, all percentages by weight, were prepared in the same manner as set forth in Example 1.

The test bars of this example had a rupture life in excess of 51 hours under a load of 15,000 p.s.i. at a temperature of about 1800° F. in air.

#### Example 12

A 5 pound alloy melt and test bars of the same dimensions as set forth in Example 1 of a cobalt base metal alloy composition containing about 19 percent of chromium, about 7.7 percent of tungsten, about 6.7 percent of tantalum, about 0.05 percent of titanium, about 0.88 percent of carbon, about 0.1 percent of silicon, about 0.05 percent of nickel, about 0.48 percent of iron, about 0.1 percent of manganese, and the balance essentially cobalt, all percentages by weight, were prepared in the same manner as set forth in Example 1.

The test bars of this example had an elongation of 75

about 3.3 percent at room temperature under a tensile stress of 142,800 p.s.i.

The test bars of this example had a rupture life in excess of 51 hours under a load of 15,000 p.s.i. at a temperature of about 1800° F. in air and a rupture life in excess of 137 hours under a load of 20,000 p.s.i. at a temperature of about 1700° F. in air.

#### Example 13

10 A 5 pound alloy melt and test bars of the same dimensions as set forth in Example 1 of a cobalt base metal alloy composition containing about 20 percent of chromium, about 10 percent of tungsten, about 10 percent of tantalum, about 0.9 percent of carbon, about 0.3 percent of silicon, about 0.5 percent of manganese, about 0.5 percent of titanium, and the balance essentially cobalt, all percentages by weight, were prepared in the same manner as set forth in Example 1.

15 The test bars of this example had an elongation of 2.5 percent at room temperature under a tensile stress of 139,000 p.s.i.

20 The test bars of this example had a rupture life in excess of 60 hours under a load of 22,500 p.s.i. at a temperature of about 1700° F. in air and a rupture life in excess of 41 hours under a load of 17,000 p.s.i. at a temperature of about 1800° F. in air.

#### Example 14

25 A 5 pound alloy melt and test bars of the same dimensions as set forth in Example 1 of a cobalt base metal alloy composition containing about 20 percent of chromium, about 7.5 percent of tungsten, about 7.5 percent of tantalum, about 0.1 percent of titanium, about 0.85 percent of carbon, about 0.01 percent of boron, and the balance essentially cobalt, all percentages by weight, were prepared in the same manner as set forth in Example 1.

30 The test bars of the example had an elongation of 1.6 percent at room temperature under a tensile stress of 142,200 p.s.i.

35 The test bars of this example had a rupture life in excess of 134 hours under a load of 22,500 p.s.i. at a temperature of about 1700° F. in air and a rupture life in excess of 51 hours under a load of 17,000 p.s.i. at a temperature of about 1800° F. in air.

#### Example 15

40 A 5 pound alloy melt and test bars of the same dimensions as set forth in Example 1 of a cobalt base metal alloy composition containing about 15 percent of chromium, about 10 percent of tungsten, about 10 percent of tantalum, about 0.1 percent of titanium, about 0.85 percent of carbon, about 0.01 percent of boron, about 5 percent of nickel, and the balance essentially cobalt, all percentages by weight, were prepared in the same manner as set forth in Example 1.

45 The test bars of this example had an elongation of 2.5 percent at room temperature under a tensile stress of 125,600 p.s.i.

50 The test bars of this example had a rupture life in excess of 166 hours under a load of 22,500 p.s.i. at a temperature of about 1700° F. in air and a rupture life in excess of 68 hours under a load of 17,000 p.s.i. at a temperature of about 1800° F. in air.

#### Example 16

55 A 5 pound alloy melt and test bars of the same dimensions as set forth in Example 1 of a cobalt base metal alloy composition containing about 22 percent of chromium, about 10 percent of tungsten, about 10 percent of tantalum, about 0.1 percent of titanium, about 0.85 percent of carbon, about 0.01 percent of boron, about 5 percent of iron, and the balance essentially cobalt, all percentages by weight, were prepared in the same manner as set forth in Example 1.

60 The test bars of this example had an elongation of 1.6

percent at room temperature under a tensile stress of 137,500 p.s.i.

The test bars of this example had a rupture life in excess of 59 hours under a load of 15,000 p.s.i. at a temperature of about 1800° F. in air and a rupture life in excess of 30 hours under a load of 8,000 p.s.i. at a temperature of about 2000° F. in air.

*Example 17*

A 5 pound alloy melt and test bars of the same dimensions as set forth in Example 1 of a cobalt base metal alloy composition containing about 22 percent of chromium, about 10 percent of tungsten, about 10 percent of tantalum, about 0.1 percent of titanium, about 0.85 percent of carbon, about 0.01 percent of boron, about 5 percent of nickel, and the balance essentially cobalt, all percentages by weight, were prepared in the same manner as set forth in Example 1.

The test bars of this example had an elongation of 3.3 percent at room temperature under a tensile stress of 134,900 p.s.i.

The test bars of this example had a rupture life in excess of 56 hours under a load of 15,000 p.s.i. at a temperature of about 1800° F. in air and a rupture life in excess of 25 hours under a load of 8,000 p.s.i. at a temperature of about 2000° F. in air.

*Example 18*

A 5 pound alloy melt and test bars of the same dimensions as set forth in Example 1 of a cobalt base metal alloy composition containing about 22 percent of chromium, about 10 percent of tungsten, about 10 percent of tantalum, about 0.1 percent of titanium, about 1.3 percent of carbon, and 0.01 percent of boron, and the balance essentially cobalt, all percentages by weight, were prepared in the same manner as set forth in Example 1.

The test bars of this example had an elongation of 1.7 percent at room temperature under a tensile stress of 145,500 p.s.i.

The test bars of this example had a rupture life in excess of 41 hours under a load of 15,000 p.s.i. at a temperature of about 1800° F. in air.

*Example 19*

A 5 pound alloy melt and test bars of the same dimensions as set forth in Example 1 of a cobalt base metal alloy composition containing about 22 percent of chromium, about 10 percent of tungsten, about 10 percent of tantalum, about 0.1 percent of titanium, about 0.2 percent of boron, about 0.85 percent of carbon, and the balance essentially cobalt, all percentages by weight, were prepared in the same manner as set forth in Example 1.

The test bars of this example had an elongation of 0.8 percent at room temperature under a tensile stress of 135,000 p.s.i.

The test bars of this example had a rupture life in excess of 50 hours under a load of 15,000 p.s.i. at a temperature of about 1800° F. in air.

*Example 20*

A 5 pound alloy melt and test bars of the same dimensions as set forth in Example 1 of a cobalt base metal alloy composition containing about 22 percent of chromium, about 8 percent of tungsten, about 8 percent of tantalum, about 3 percent of columbium, about 0.1 percent of titanium, about 0.85 percent of carbon, about 0.01 percent of boron, and the balance essentially cobalt, all percentages by weight, were prepared in the same manner as set forth in Example 1.

The test bars of this example had an elongation of 0.95 percent at room temperature under a tensile stress of 125,000 p.s.i.

The test bars of this example had a rupture life in excess of 62 hours under a load of 15,000 p.s.i. at a temperature of about 1800° F. in air.

*Example 21*

A 5 pound alloy melt and test bars of the same dimensions as set forth in Example 1 of a cobalt base metal alloy composition containing about 22 percent of chromium, about 12.5 percent of tungsten, about 3 percent of tantalum, about 1 percent of columbium, about 0.1 percent of titanium, about 1 percent of carbon, about 0.01 percent of boron, and the balance essentially cobalt, all percentages by weight, were prepared in the same manner as set forth in Example 1.

The test bars of this example had an elongation of .8 percent at room temperature under a tensile stress of 137,000 p.s.i.

The test bars of this example had a rupture life in excess of 22 hours under a load of 15,000 p.s.i. at a temperature of about 1800° F. in air.

*Example 22*

A 5 pound alloy melt and test bars of the same dimensions as set forth in Example 1 of a cobalt base metal alloy composition containing about 22 percent of chromium, about 12.5 percent of tungsten, about 3 percent of tantalum, about 1 percent of columbium, about 0.1 percent of titanium, about 1 percent of carbon, about 0.01 percent of boron, about 5 percent of nickel, and the balance essentially cobalt, all percentages by weight, were prepared in the same manner as set forth in Example 1.

The test bars of this example had an elongation of 3 percent at room temperature under a tensile stress of 131,900 p.s.i.

The test bars of this example had a rupture life in excess of 41 hours under a load of 15,000 p.s.i. at a temperature of about 1800° F. in air.

*Example 23*

A 5 pound alloy melt and test bars of the same dimensions as set forth in Example 1 of a cobalt base metal alloy composition containing about 22 percent of chromium, about 8 percent of tungsten, about 8 percent of tantalum, about 1 percent of columbium, about 0.1 percent of titanium, about 0.85 percent of carbon, about 0.01 percent of boron, and the balance essentially cobalt, all by weight, were prepared in the same manner as set forth in Example 1.

The test bars of this example had an elongation of 1.6 percent at room temperature under a tensile stress of 132,100 p.s.i.

The test bars of this example had a rupture life in excess of 277 hours under a load of 20,000 p.s.i. at a temperature of about 1700° F. in air, a rupture life in excess of 128 hours under a load of 15,000 p.s.i. at a temperature of about 1800° F. in air.

*Example 24*

A 5 pound alloy melt and test bars of the same dimensions as set forth in Example 1 of a cobalt base metal alloy composition containing about 22 percent of chromium, about 8 percent of tungsten, about 8 percent of tantalum, about 1 percent of columbium, about 0.1 percent of titanium, about 0.85 percent of carbon, about 0.01 percent of boron, about 5 percent of iron, and the balance essentially cobalt, all percentages by weight, were prepared in the same manner as set forth in Example 1.

The test bars of this example had an elongation of 0.8 percent at room temperature under a tensile stress of 127,600 p.s.i.

The test bars of this example had a rupture life in excess of 33 hours under a load of 15,000 p.s.i. at a temperature of about 1800° F. in air and a rupture life in excess of 19 hours under a load of 5,000 p.s.i. at a temperature of about 2000° F. in air.

*Example 25*

A 5 pound alloy melt and test bars of the same dimensions

sions as set forth in Example 1 of a cobalt base metal alloy composition containing about 25 percent of chromium, about 10 percent of tungsten, about 5 percent of tantalum, about 2 percent of columbium, about 0.85 percent of carbon, about 0.1 percent of titanium, about 0.01 percent of boron, about 5 percent of iron, and the balance essentially cobalt, all percentages by weight, were prepared in the same manner as set forth in Example 1.

The test bars of this example had an elongation of 1.6 percent at room temperature under a tensile stress of 139,400 p.s.i.

The test bars of this example had a rupture life in excess of 53 hours under a load of 15,000 p.s.i. at a temperature of about 1800° F. in air and a rupture life in excess of 21 hours under a load of 5,000 p.s.i. at a temperature of about 2000° F. in air. The oxidation penetration was 0.017 mil per side per hour after 100 hours in moving air at 2000° F. and 0.07 mil per side per hour after 24 hours in moving air at 2100° F.

#### Example 26

A 5 pound alloy melt and test bars of the same dimensions as set forth in Example 1 of a cobalt base metal alloy composition containing about 18 percent of chromium, about 8.6 percent of tungsten, about 2.5 percent of tantalum, about 0.6 percent of titanium, about 0.1 percent of zirconium, about 0.49 percent of carbon, about 0.2 percent of silicon, about 2.5 percent of nickel, about 2.5 percent of iron, and the balance essentially cobalt, all percentages by weight, were prepared in the same manner as set forth in Example 1.

The test bars of this example had an elongation of 3 percent at room temperature under a tensile stress of 100,000 p.s.i.

The test bars of this example had a rupture life in excess of 250 hours under a load of 22,000 p.s.i. at a temperature of about 1600° F. in air and a rupture life in excess of 100 hours under a load of 10,000 p.s.i. at a temperature of about 1800° F. in air.

#### Example 27

A 5 pound alloy melt and test bars of the same dimensions as set forth in Example 1 of a cobalt base metal alloy composition containing about 20 percent of chromium, about 11 percent of tungsten, about 0.5 percent of tantalum, about 2.9 percent of titanium, about 0.1 percent of zirconium, about 0.7 percent of carbon, about 0.4 percent of silicon, about 0.5 percent of nickel, about 0.5 percent of iron, and the balance essentially cobalt, all percentages by weight, were prepared in the same manner as set forth in Example 1.

The test bars of this example had an elongation of 8 percent at room temperature under a tensile stress of 115,000 p.s.i.

The test bars of this example had a rupture life in excess of 100 hours under a load of 15,000 p.s.i. at a temperature of about 1700° F. in air and a rupture life in excess of 100 hours under a load of 10,000 p.s.i. at a temperature of about 1800° F. in air.

The above detailed description has been given for clearness of understanding only. No unnecessary limitations should be understood therefrom, as modifications will be obvious to those skilled in the art.

I claim:

1. A metal alloy consisting essentially of, by weight, from about 15 to about 28 percent of chromium, from about 5 to about 15 percent of tungsten, from about 0.5 to about 20 percent of tantalum, from about 0.01 to about 3 percent of titanium, from about 0.6 to about 1.3 percent of carbon, and the balance cobalt.

2. A metal alloy consisting essentially of, by weight, from about 16 to about 25 percent of chromium, from about 7.5 to about 12.5 percent of tungsten, from about 7

to about 11 percent of tantalum, from about 0.08 to about 0.5 percent of titanium, from about 0.6 to about 1 percent of carbon, and the balance cobalt.

3. A metal alloy consisting essentially of, by weight, from about 15 to about 28 percent of chromium, from about 5 to about 15 percent of tungsten, from about 0.5 to about 20 percent of tantalum, up to about 3 percent of columbium, with the columbium content not more than about 50 percent of the amount of tantalum in the alloy, from about 0.01 to about 3 percent of titanium, from about 0.6 to about 1.3 percent of carbon, and the balance cobalt.

4. A metal alloy consisting essentially of, by weight, from about 15 to about 28 percent of chromium, from about 5 to about 15 percent of tungsten, from about 0.5 to about 20 percent of tantalum, from about 0.01 to about 3 percent of titanium, up to about 3.5 percent of molybdenum, with the molybdenum content not more than about 50 percent of the amount of tungsten in the alloy, from about 0.6 to about 1.3 percent of carbon, and the balance cobalt.

5. A metal alloy consisting essentially of, by weight, from about 15 to about 28 percent of chromium, from about 5 to about 15 percent of tungsten, from about 0.5 to about 20 percent of tantalum, from about 0.01 to about 3 percent of titanium, up to about 0.2 percent of boron, from about 0.6 to about 1.3 percent of carbon, and the balance cobalt.

6. A metal alloy consisting essentially of, by weight, from about 15 to about 28 percent of chromium, from about 5 to about 15 percent of tungsten, from about 0.5 to about 20 percent of tantalum, up to about 3 percent of columbium, with the columbium content not more than about 50 percent of the amount of tantalum in the alloy, from about 0.01 to about 3 percent of titanium, zirconium in an amount such that, if the amount of titanium is more than 0.5 percent, the combined amount of titanium and zirconium is equal to or less than 3 percent, and if the amount of titanium is equal to or less than 0.5 percent, titanium is more than about 70 percent of zirconium, up to about 0.2 percent of boron, up to about 3.5 percent of molybdenum, with the molybdenum content not more than about 50 percent of the amount of tungsten in the alloy, from about 0.6 to about 1.3 percent of carbon, and the balance cobalt.

7. A metal alloy consisting essentially of, by weight, from about 15 to about 28 percent of chromium, from about 5 to about 15 percent of tungsten, from about 0.5 to about 20 percent of tantalum, from about 0.01 to about 3 percent of titanium, zirconium in an amount such that, if the amount of titanium is more than 0.5 percent, the combined amount of titanium and zirconium is equal to or less than 3 percent, and if the amount of titanium is equal to or less than 0.5 percent, titanium is more than about 70 percent of the zirconium, from about 0.6 to about 1.3 percent of carbon, up to about 1.5 percent of silicon, up to about 5 percent of nickel, up to about 5 percent of iron, and the balance cobalt.

8. A metal alloy consisting essentially of, by weight, from about 15 to about 28 percent of chromium, from about 5 to about 15 percent of tungsten, from about 0.5 to about 20 percent of tantalum, up to about 3 percent of columbium, with the columbium content not more than about 50 percent of the amount of tantalum in the alloy, from about 0.01 to about 3 percent of titanium, zirconium in an amount such that, if the amount of titanium is more than 0.5 percent, the combined amount of titanium and zirconium is equal to or less than 3 percent, and if the amount of titanium is equal to or less than 0.5 percent, titanium is more than about 70 percent of the zirconium, up to about 0.2 percent of boron, up to about 3.5 percent of molybdenum, with the molybdenum content not more than about 50 percent of the amount of tungsten in the alloy, from about 0.6 to about 1.3 percent of carbon, up to about 1.5 percent of silicon, up

**11**

to about 5 percent of nickel, up to about 5 percent of iron and the balance cobalt.

9. A metal alloy consisting essentially of, by weight, from about 16 to about 25 percent of chromium, from about 7.5 to about 12.5 percent of tungsten, up to about 3.5 percent of molybdenum, from about 7 to about 11 percent of tantalum, up to about 3 percent of columbium, from about 0.08 to about 0.5 percent of titanium, zirconium in an amount such that the amount of titanium is more than 70 percent, the amount of zirconium in the alloy, from about 0.6 to about 1 percent of carbon, up to about 0.2 percent of boron, up to about 1.5 percent of silicon, up to about 2.5 percent of nickel, up to about 2.5 percent of iron, and the balance cobalt.

**12**

2,515,774 Johnson \_\_\_\_\_ July 18, 1950  
 2,684,299 Binder \_\_\_\_\_ July 20, 1954  
 2,771,360 Malcolm \_\_\_\_\_ Nov. 20, 1956

## FOREIGN PATENTS

5 443,821 Great Britain \_\_\_\_\_ Mar. 6, 1936  
 686,180 Great Britain \_\_\_\_\_ Jan. 21, 1953  
 542,813 Canada \_\_\_\_\_ June 25, 1957

## OTHER REFERENCES

10 Materials and Methods, September 1953; Number 260, page 139.

**15**

## References Cited in the file of this patent

## UNITED STATES PATENTS

2,247,643 Rohn et al. \_\_\_\_\_ July 1, 1941